

Aug. 7, 1945.

D. A. OLIVER

2,381,363

## MANUFACTURE OF FERRO-MAGNETIC MATERIAL

Filed Sept. 22, 1941



FIG. 3.

Nataou, Cole, Hinckle & Nataou

## UNITED STATES PATENT OFFICE

2,381,363

## MANUFACTURE OF FERROMAGNETIC MATERIAL

Donald Arthur Oliver, Sheffield, England, assignor  
to William Jessop & Sons Limited, Sheffield,  
England

Application September 22, 1941, Serial No. 411,936  
In Great Britain September 21, 1940

4 Claims. (Cl. 148—10)

(Granted under the provisions of sec. 14, act of  
March 2, 1927; 357 O. G. 5)

This invention relates to the manufacture of ferro-magnetic material by a process of the kind in which anisotropic magnetic characteristics are developed by subjecting the material to a magnetic field during cooling from an elevated temperature which is usually one above the Curie point, the object of the invention being to provide an improved process of this kind for enabling latent magnetic properties of ferro-magnetic material to be developed in a controlled manner.

More particularly the object is to enable optimum magnetic properties in such material to be developed for purposes such as the employment of the material in magneto-generators or in transformers.

Other objects are implicit in the following description of the invention.

Hitherto the anisotropy produced by subjecting ferro-magnetic material to a magnetic field during cooling from an elevated temperature has been such that the magnetic characteristics have been enhanced in one (a principal) direction only at the expense of those in all other directions but anisotropic ferro-magnetic material according to the present invention has magnetic characteristics which are enhanced in different directions in parallel planar zones, in comparison with the like characteristics in directions having a component at right angles to such planar zones. Such anisotropy may be produced by subjecting the material during cooling from a temperature above, to one below, the Curie point to a magnetic field which is concentrated along lines extending in both dimensions of such planar zones. Thus, for example, the characteristics may be enhanced, for example, along all diametrical lines of material in cylindrical or disc-like form.

The invention is particularly applicable to high coercivity material, such as for example, an iron base alloy containing 13% to 30% of cobalt, 8% to 20% of nickel and 5% to 10% of aluminium, although it may also be applied to high permeability material.

In the method of producing the desired anisotropic properties in ferro-magnetic material according to the present invention, relative rotation between the material and the magnetic field is maintained, during cooling of the material past the Curie point, about an axis at right angles to the planar zones in which the multi-directional characteristics of augmented value are to be produced. Thus the material may be rotated in the magnetic field or may be stationary in a rotating magnetic field set up by a three-phase stator system of alternating electric currents.

The relatively rotating ferro-magnetic material and field may be co-axial or units of material may be grouped around the axis of rotation.

Apparatus for maintaining the relative rotation of ferro-magnetic material and magnetic field may comprise a bi-polar magnetic system, which may be energised by a permanent magnet or magnets or by continuous or alternating electric current, a carrier mounted in bearings to rotate in a gap between polar faces of the magnetic system about an axis at right angles to the direction of the field, means for attaching the heated material to the carrier and means for rotating the latter.

15 The carrier may vary in construction according to the form or shape of the material to be treated. Thus for material having axial grooves or eccentric apertures the carrier may comprise heat resistant rods grouped around the axis of rotation and each in two portions connected by a spigot and socket joint. The heated material may be attached to the carrier by separating the rods thereof at their joints, causing them to engage the grooves or apertures in the material and re-connecting them.

20 When the material has a central aperture the carrier may comprise a mandrel and heat resistant supports projecting radially therefrom and adapted to engage the aperture in the ferro-magnetic material. In a modification a flange may project from the mandrel at right angles to the axis of rotation and means be provided for clamping the ferro-magnetic material against the flange.

25 In all cases the anisotropic character of high coercivity material manufactured according to the present invention is not impaired by subsequent demagnetisation or magnetisation in any direction and, before use, such material may be, and preferably, is re-magnetised in the desired directions in the planar zones in which its magnetic characteristics have been enhanced.

30 In the accompanying drawing:  
Figure 1 is a longitudinal section of a device according to the present invention for rotating ferro-magnetic material in a magnetic field.

35 Figure 2 is a transverse section on the line 2—2 of Figure 1.

40 Figures 3 and 4 are diagrams illustrating apparatus for carrying out the present invention.

45 Like reference numerals indicate like parts throughout the drawing.

50 With reference first to Figures 1 and 2 the device illustrated comprises two pole-pieces 10 and 11 of soft iron which are adapted to form part of

a bi-polar magnetic system as hereinafter described with reference to Figures 3 and 4.

The gap between the pole pieces 10 and 11 is enclosed by plates of non-magnetic material, one end plate 12 and the two side plates 13 and 14 being more or less permanently secured by screws 15 to the pole pieces 10 and 11 thus forming a box-like contrivance. The other end plate 16 is detachably attached in place by dowel pins 17.

In the particular example illustrated the material to be treated is in the form of a disc 18 having axial slots 19 in its periphery and a carrier for the disc 18 is rotatably mounted in ball bearings 20 and 21 respectively secured in the end plates 12 and 16. This carrier is of a cage-like construction comprising end discs or spiders 22 and 23 connected by heat resistant rods 24. Each of the rods 24 is in two portions connected by spigot and socket joints indicated at 25. The end disc 22 of the carrier has a tapered trunnion 26 detachably engaged with the inner race of the ball bearing 20 and the end disc 23 has a spindle portion 27 mounted in the inner race of the ball bearing 21 and carrying on the other side of the end plate 16 a pulley 28 by means of which the carrier may be rotated.

It will be appreciated that the pole pieces 10 and 11 are comprised in a bi-polar magnetic system which, as indicated in Figure 3, may be energized by a continuous or alternating electric current passing round the coils 29. If desired, however, the magnetic system may be energized by a permanent magnet 30 as indicated in Figure 4.

In use the end plate 16 is detached from the pole pieces 10 and 11 carrying with it the complete carrier. The carrier is then separated at the spigot and socket joints 25 of the heat resistant rods 24 and the spigots of the latter are then engaged in the grooves 19 of the disc 18 which is at a temperature above the Curie point and preferably in the neighbourhood of 1200° C. The carrier is then replaced in the gap between the pole pieces 10 and 11, this operation being facilitated by the tapered formation of the end of the trunnion 26. Whilst the temperature of the material 18 is still above the Curie point the cage is driven by power applied to the pulley 28 thereby rotating the material 18 in the magnetic field between the pole pieces 10 and 11.

In a particular example a disc of high coercive material consisting of an iron base alloy containing 24.9% of cobalt, 11.1% of nickel, 6.8% of aluminum, 2.3% of copper, 0.03% of carbon, and 2.1% of titanium, was cast in disc form which was raised to a temperature of 1200° C., placed in the device illustrated in Figures 1 and 2 and rotated at a speed of 600 revolutions per minute in a magnetic field strength of 5,000 oersted until cooled to a temperature of about 600° C. The disc was then removed from the apparatus and was found to possess in all directions in the plane of the disc a remanence of 10,000 gauss, a coercive force of 450 oersteds and a  $(BH)_{max}$  of 2,000,000. Measured in an axial di-

rection the disc possessed a remanence of 2,000 gauss, a coercive force of 220 oersteds and a  $(BH)_{max}$  of 820,000.

A sample of the same alloy possessing isotropic magnetic characteristics (i. e. heat treated without the influence of a magnetic field to give optimum properties) has a remanence of 9,000 gauss, a coercive force of 50 oersteds and a  $(BH)_{max}$  of 180,000. Thus the treatment of a cylindrical body in the apparatus described above according to the present invention results in augmenting the magnetic values along all diameters of any section perpendicular to the axis in comparison not only with the values in the direction of the axis of that body but also with the values in any direction of an isotropic body of the same material.

What I claim is:

1. The method of producing anisotropic properties in ferro-magnetic material such that magnetic characteristics are enhanced in different directions in parallel planar zones, in comparison with the like characteristics in directions having a component at right angles to such planar zones, by subjecting the material during cooling from a temperature above to one below the Curie point to a magnetic field and by maintaining relative rotation between the material and the magnetic field, during cooling of the material past the Curie point, about an axis at right angles to the planar zones in which the multi-directional characteristics of augmented value are to be produced.

2. The method as in claim 1 in which the material is rotated in the magnetic field.

3. The method of producing anisotropic properties in ferro-magnetic material such that magnetic characteristics are enhanced in different directions in parallel planar zones, in comparison with the like characteristics in directions having a component at right angles to such planar zones, by subjecting the material during cooling from a temperature above to one below the Curie point to a rotating magnetic field set up by a three-phase stator system of alternating electric currents causing the said field to rotate about an axis at right angles to the planar zone in which the multi-directional characteristics of augmented value are to be produced.

4. The method of producing anisotropic properties in high coercivity material consisting of an iron base alloy containing 13% to 30% of cobalt, 8% to 20% of nickel and 5% to 10% of aluminum by subjecting a body of such alloy during cooling from a temperature above to one below the Curie point to a magnetic field and by maintaining relative rotation between the said body and the magnetic field, during cooling of the body past the Curie point, about an axis at right angles to the planar zones in which the multi-directional characteristics of augmented value are to be produced.

DONALD ARTHUR OLIVER.